

# UNITED STATES PATENT OFFICE.

JEAN ROSEN, OF PARIS, FRANCE.

## PROCESS FOR THE MANUFACTURE OF A PLASTIC AND ELASTIC MATERIAL FOR TARRING ROADS OR FOR OTHER PURPOSES.

1,155,442.

Specification of Letters Patent.

Patented Oct. 5, 1915.

No Drawing.

Application filed August 8, 1913. Serial No. 783,814.

To all whom it may concern:

Be it known that I, JEAN ROSEN, citizen of France, residing at Paris, France, have invented new and useful Improvements in 5 Process for the Manufacture of a Plastic and Elastic Material for Tarring Roads or for other Purposes, of which the following is a specification.

The tarring of roads and preparation of 10 macadam or road coverings of tarred stones is usually effected with coal tar, the physical properties of which are hardly examined, provided the tar is sufficiently viscid to act as a binder. It has been found that the 15 kinds of coal tar that are usually used do not properly resist the general use and traffic of the road, owing to the fact that they are inclined to become brittle, as they contain naphthalene, which imparts a strongly crystalline structure to the tar. It has also been 20 observed that the phenols that are found in coal tar produce a very noxious effect on plants and on the feet of animals. Tar on the other hand from which naphthalene and 25 phenols have been withdrawn, could hardly be used for tarring roads because the coating obtained in such case would not be sufficiently soft and flexible and would become brittle, owing to the oxidizing effect pro- 30 duced by the air and warm weather. The present invention is intended to avoid this drawback and produce tar that has a maximum amount of consistency and tenacity although it is deprived of phenols and naphthalene *i. e.*, the constituents referred to 35 above as having a detrimental effect.

According to the principle of this invention the naphthalene and excess of naphthalene oils (3 to 20%) as well as the phenols 40 and phenol oils of the tar are withdrawn, and oils are then added that impart a much greater consistency and tenacity to the tar. It is not my desire to protect any particular process for withdrawing the deleterious 45 substances from the tar, since I may withdraw them in any suitable manner before adding anthracene and anthracene oils which are particularly beneficial to compounds of this character. By way of sug- 50 gestion, the phenols can be withdrawn in the following manner:—First heat coal tar to a temperature varying from 150° C. to 200° C. and then treat the heated coal tar with caustic soda which dissolves the phenol 55 and its homologues together with a certain

quantity of naphthalene and other hydrocarbons. The solution is then distilled with water and the hydro-carbons are thereby precipitated and separated. Then the solution is acidified and the phenols are liberated and form an oily layer on the surface of the acid. There are a number of other ways in which phenol may be separated from coal tar, but this method is offered as a suggestion of a way in which it may be 60 done with a separation of naphthalene also taking place. Naphthalene may be separated from the mass thereafter by first boiling the mass at a temperature varying from 270° C. to 400° C., and then allowing the 65 same to stand for some time when it partially solidifies, and in then separating by the use of a centrifugal separating machine. The lower melting point impurities are freed by means of hot water, and the residue is finally hot pressed. The crude anthracene cake is purified by treatment with pyridin bases and the whole can be dissolved on heating and the anthracene 70 crystallized on cooling, and the anthracene 75 crystals then removed centrifugally. I disclaim this specific process of withdrawing the detrimental substances from the tar since it is well known and is not my invention. This 80 result is obtained by using anthracene and 85 anthracene oils that are added to the mass of tar when the latter has been deprived of the excess of the products that produce a crystalline structure and give it a caustic 90 effect. The tar is brought to a temperature 95 between 90° C. and 200° C., before adding the anthracene and anthracene oils, and the mixture is then thickened by means of a current of air until the material treated has 100 attained the required consistency, which can be carried as far if necessary as that of a solid material. This oxidation which leads to a definite physical state has the advantage moreover of producing a material, that is far less sensitive to effects of subsequent 105 oxidation and therefore retains its plastic properties. The mass prepared in this manner is no longer brittle, as it no longer contains the products that caused this drawback and as materials have been added to the same that increase its viscid and flexible properties. The mass obtained is moreover amorphous and deprived of obnoxious crystals. The road coverings obtained with tars 110 of this kind that have already been oxidized,

no longer tend to become brittle, even if the roads on which this kind of tar is used have to stand a great deal of traffic and considerable variations of temperature. These 5 coverings are far more resistant and durable than the road coverings hitherto prepared with ordinary tar. The quantity of anthracene added may be such that the mixture to be oxidized may contain up to 90% 10 of anthracene.

What I claim is:

1. A process for the manufacture of plastic material consisting in treating coal tar to remove phenols and phenol oils and 15 naphthalene and naphthalene oils from the coal tar, then mixing anthracene and anthracene oils with the residue, and then oxidizing the mixture to provide a viscous and flexible compound.
- 20 2. A process for the manufacture of plastic material consisting in withdrawing from coal tar the phenols and phenol oils which are detrimental because of their caustic effect and separating naphthalene and naphthalene oils because of the crystalline struc- 25

ture which they impart to the composition which contains them, adding anthracene and anthracene oils to the residue thus prepared while the same is in a heated state, and subsequently applying a current of air 30 to the mixture to render it viscous.

3. A process for the manufacture of plastic material consisting in withdrawing from coal tar the phenols and phenol oils which are detrimental because of their caustic effect and separating naphthalene and naphthalene oils because they impart a crystalline structure thereto, then adding anthracene and anthracene oils to the residue while the same is heated to a temperature between 30 90° C. and 200° C., and subsequently passing a current of air through the same so as to thicken the mixture and render it viscous.

In testimony whereof I have signed my name to this specification in the presence 45 of two subscribing witnesses.

JEAN ROSEN.

Witnesses:

L. FEITLINE,  
LUCIEN MEMMINGER.